

F. D. & E. D. BELKNAP.

STENCIL CARD OR SHEET AND PROCESS OF PRODUCING SAME.

APPLICATION FILED JUNE 2, 1910.

1,110,869.

Patented Sept. 15, 1914.

Fig. 1.



Fig. 2.



Fig. 3.



Witnesses:  
M. H. Crawford  
L. Samuels

Inventors  
Frank D. Belknap  
Edmund D. Belknap  
By the Attorney  
W. Park Reinharts

# UNITED STATES PATENT OFFICE.

FRANK D. BELKNAP, OF NEW YORK, N. Y., AND EDWIN DRAYTON BELKNAP, OF EAST ORANGE, NEW JERSEY.

## STENCIL CARD OR SHEET AND PROCESS OF PRODUCING SAME.

1,110,869.

Specification of Letters Patent.

Patented Sept. 15, 1914.

Application filed June 2, 1910. Serial No. 564,619.

*To all whom it may concern:*

Be it known that we, FRANK D. BELKNAP and EDWIN D. BELKNAP, citizens of the United States of America, residing at New York city, county and State of New York, and East Orange, county of Essex, State of New Jersey, respectively, have invented certain new and useful Improvements in Stencil Cards or Sheets and Process of Producing Same, of which the following is a specification.

Our invention comprises an improved stencil card or sheet capable of being stencilized and process of making same.

Our invention is principally used in producing duplicate copies of typewritten matter. Sheets of paper embodying our invention are treated in such manner that when struck or stamped with a type or other block having a character or design formed thereon in raised portions, the said character or design is indented in the film of material with which the paper has been treated, leaving the loosely felted fiber of the paper intact. The paper so treated becomes a perfect stencil through which printing ink may be forced upon an underlying sheet of paper and produce a perfect facsimile of the original character or design appearing on the type, exactly as though the type or engraved block had been inked in the usual way and pressed upon the paper in an ordinary printing operation, or any ink ribbon used.

In carrying out our process we take the thin paper known as Japanese paper or other thin paper of similarly loose texture and subject it to treatment with some or all of the following solutions: First, a solution of from 1 to 2 ounces of gelatin in about a quart of water. Second, an ounce of bichromate of potash dissolved in about three quarts of water. Third, a mixture of one pint of formaldehyde and one pint of water. Fourth, a mixture of about 18 ounces of glycerin and 8 ounces of sugar and enough water to fill a quart measure with the solution thus formed.

The first solution is preferably formed with hot water. The sheet of paper may be

dipped in the solutions separately and consecutively, or the last three solutions may be mixed together and the paper dipped in the resulting liquid. Whether some or all of the solutions mentioned are employed, it is essential that gelatin, or other equivalent colloid be used, this forming the main body of the coating film to be produced and also that such coating film, after deposition, be subjected to the action of a coagulating agent such as an alkaline bichromate, or formaldehyde. Also, as applicants' practice is to carry out that process in daylight, the materials must be separated into at least two solutions, one including the gelatin or other colloid, and the other solution including the coagulating agent, and that the dipping in, or other treatment by these two solutions, should be successive, treatment with the colloid solution being preferably done first. It is evident that if the colloid and the coagulant were mixed in one solution before application to the paper, or if the paper were treated simultaneously with the colloid solution and the coagulating solution, the colloid would be wholly or partly coagulated before it could be distributed in an even film over the paper, (unless the coagulating action were extremely slow) and the coating so formed would be uneven and full of pin holes. It is therefore advisable that the paper first be treated with the colloid solution, so that it may form an even, imperforate film or coating thereon, and that this coating film be subsequently coagulated, or fixed, by treatment with the coagulating solution. The paper known as Japanese dental paper or Yoshino gives good results. After dipping, the paper is then dried, or if stencil cards are to be made of it, the paper is laid over suitable cardboard frames and cemented or otherwise fastened thereto. The solution itself may serve as the cement.

In the accompanying drawing, Fig. 1 represents a piece of card board cut out to form a series of frames for a series of cards. Fig. 2 shows a sheet of treated paper fastened thereto, and Fig. 3 shows a detached card.

Throughout the drawings like reference numerals indicate like parts.

1 is the treated sheet of paper, 2 is the strip of cardboard cut out at 3, 3, to form the frames, and 1<sup>a</sup> is the portion of paper and 2<sup>a</sup> the portion of cardboard forming a single card.

The card so formed is put in an ordinary typewriter, preferably provided with the attachment shown in Patent No. 960,252 issued to Frank D. Belknap June 7, 1910, and the name and address of a person, or any other desired matter is written thereon by operating the typewriter in the same way as is done in forming ordinary wax paper stencils. When the cards so formed and treated are put through any suitable stencil printing apparatus, such as is shown for instance in Patent No. 889,503, issued to Edwin D. Belknap, the ink goes through the portions of the paper against which the type faces have struck, and not through the other portions. The result is a perfect printing on the envelopes or other articles run through the machine concurrently with the cards. The printing so performed can not be distinguished from printing done directly by the same typewriting machine in the ordinary way. The paper so treated resists the action of the atmosphere, adheres closely to the ordinary cardboard frame, and seems to expand and contract under variations of heat and moisture at about the same rate as the cardboard frame so that the card does not buckle or curl in use.

We have made many experiments with the ordinary waxed papers on the market in the effort to make satisfactory stencil cards of this kind, and have experimented with many different solutions and fillers in the effort to produce an absolutely satisfactory stencil card for use in addressing machines, but the materials above described are the first to give perfectly satisfactory results. The treated paper is more like a parchment paper than like the ordinary waxed stencil paper.

The coagulated gelatin or other colloid forms the basis of the coating film, giving it the necessary strength and coherency, while the glycerin is an example of a tempering agent which, by its admixture in regulated quantities, prevents the coagulated colloidal films from becoming too hard, or otherwise resisting the displacing pressure of the type to too great an extent.

While the best results are obtained by the treatment with all of the solutions described, less perfect results may be obtained by using some of the materials without the other. The best results are also obtained if the stencil sheet is run through the typewriter while slightly damp. When the sheet is not stencilized until after it has become dry,

this dampening may be effected by going over the face of the sheet with a wet brush. Other alkaline bichromates can be substituted for the bichromate of potash particularly above mentioned.

Having, therefore, described our invention, we claim:

1. As a new article of manufacture, a stencil sheet for use in producing duplicate copies of typewritten matter which consists of a thin sheet of paper of loose texture, treated with successive solutions of gelatin, glycerin and bichromate of potash and having the characters to be reproduced indented in the film of treating solution carried by said paper, the paper being left intact. 80

2. As a new article of manufacture, a stencil sheet for use in producing duplicate copies of typewritten matter which consists of a thin sheet of paper of loose texture, treated with successive solutions of gelatin, glycerin and an alkaline bichromate and having the characters to be reproduced indented in the film of treating solution carried by said paper, the paper being left intact. 90

3. As a new article of manufacture, a stencil sheet for use in producing duplicate copies of typewritten matter which consists of a thin sheet of paper of loose texture, treated with successive solutions of gelatin, glycerin and bichromate of potash and cut in such form as to be adapted to be placed in a typewriter. 95

4. As a new article of manufacture, a stencil sheet for use in producing duplicate copies of typewritten matter which consists of a thin sheet of paper of loose texture treated with successive solutions of gelatin, glycerin and bichromate of potash and mounted on a frame adapted to be placed in a typewriter. 100

5. The process of forming a sheet for use in the production of stencils by type pressure which includes the following steps: first, depositing an even film of colloidal material on a thin loose fibered paper, and second, subjecting said film to the action of a coagulant. 110

6. The process of forming a sheet capable of being stencilized which includes saturating a thin, loose fibered paper with a solution containing gelatin, and afterward subjecting said saturated sheet to the action of a coagulant. 115

7. The process of forming a sheet capable of being stencilized which includes saturating a thin, loose fibered paper with a solution containing gelatin and a tempering agent, and afterward subjecting said saturated sheet to the action of a coagulant. 120

8. The process of forming a sheet capable of being stencilized which includes saturating a thin, loose fibered paper with a solution

containing gelatin and glycerin, and afterward subjecting said saturated sheet to the action of a coagulant.

9. The process of producing a stencil sheet capable of reproducing typewriting which includes the following steps: first, saturating a sheet of thin, loose fibered paper with a colloid solution; second, subjecting said

saturated sheet to the action of a coagulant, and, third, subjecting said sheet while damp to type pressure.

FRANK D. BELKNAP.

EDWIN DRAYTON BELKNAP.

Witnesses:

E. G. PAYSON,

CONSTANT M. EAKIN.